

Patented Nov. 14, 1922.

1,435,875

# UNITED STATES PATENT OFFICE.

CHARLES H. PROCTOR, OF ARLINGTON, AND CHRISTIAN JOHN WERNLUND, OF WOODBRIDGE TOWNSHIP, MIDDLESEX COUNTY, NEW JERSEY, ASSIGNEES TO THE ROESSLER & HASSSLACHER CHEMICAL COMPANY, A CORPORATION OF NEW YORK.

## ELECTROPLATING WITH ALKALINE BATH.

No Drawing.

Application filed December 27, 1921. Serial No. 525,128.

To all whom it may concern:

Be it known that we, CHARLES HENRY PROCTOR and CHRISTIAN JOHN WERNLUND, citizens of the United States, and residents 5 of Arlington, county of Hudson, State of New Jersey, and township of Woodbridge, in the county of Middlesex and State of New Jersey, respectively, have invented certain new and useful Improvements in Electroplating with Alkaline Bath, of which the following is a specification.

This invention relates to electroplating with zinc, and particularly to a process heretofore disclosed by us in an earlier application 15 wherein a salt of mercury is added to an alkaline bath containing cyanide for raising the cathode potential and thereby materially increasing the throwing power of such baths as compared with baths previously known. The result of this is to obtain better coatings and also to enable cast iron and irregular or recessed articles to be plated with zinc, which had heretofore been considered impracticable to be plated electrolytically, or only with considerable difficulty.

The object of the present invention is to provide an improved method and apparatus and bath for introducing the mercury 30 into the solution and maintaining it there in substantially constant amount necessary to obtain the result desired, over a considerable period of time.

We have discovered that this object can be accomplished by incorporating the mercury in a predetermined percentage in the 35 anode, constituting in effect a mercury-zinc alloy anode which is much superior either to an amalgamated zinc anode, or to the periodic replenishment of the mercury in the bath by addition of soluble mercury salts.

By this invention, using a mercury-zinc alloy anode wherein the mercury is predetermined of about one per cent, we have 45 found that the bath can be operated without attention for upwards of a month and that the percentage of mercury therein after a few hours' run is substantially the same at the end of a month or more. The practical 60 advantage is that the operator is not required to test the mercury content of the bath from time to time, nor to add mercury salts and yet the operating conditions and the results remain practically constant

throughout a long period. While our experiments have not determined the ultimate operating period of such a bath automatically replenished from the anode, we have found that in runs of over a month the percentage of mercury in solution is varied 60 within less than 15% of that found in the bath after the initial run of a few hours necessary to bring it up to working strength, and that such variation does not materially affect the results. 65

For example, in one test extending over a period of over a month using a zinc anode alloyed with 1% mercury, at the end of the initial eight-hours' run the bath contained approximately .024% of mercury and after 70 over a month's use contained approximately .021% of mercury, without appreciable variation in results. In all cases, the throwing power of such a solution was found to be very materially increased over previous 75 alkaline plating baths containing cyanide without mercury, and the mercury was found to have the effect of increasing the over voltage of the cathode, the result of which is to decrease the amount of hydrogen 80 on the cathode.

In carrying out the invention, the article to be plated is first cleaned of both oxide, oil, grease, etc., by well understood methods including sand blasting, weak acid or 85 pickling, soda, etc., to expose a clean surface, and is then immediately suspended from the cathode rod, or in a cathode basket in the plating solution. The following bath gives 90 good results:

|                 |        |
|-----------------|--------|
| Water           | 1 gal. |
| Zinc cyanide    | 4 oz.  |
| Sodium cyanide  | 4 oz.  |
| Sodium hydroxid | 2 oz.  |

The anode consists of a pure form of zinc, such as electrolytic alloyed with about 1% of mercury. We prefer to use one per cent, but this percentage can be increased or decreased according to conditions. 100

Instead of bringing up the desired concentration of mercury in the bath by solution from the anode we can add to the above bath when made up  $\frac{1}{10}$  oz. of mercuric oxide or other salt of mercury, or the equivalent 105 in mercury, per gallon, which is preferred by us rather than to bring up the desired mercury content by solution from the anode.

The solution is maintained at a temperature of from 40° to 50° C. and the preferred voltage is from three to six volts, depending upon the quantity of work being plated.

5 When the required deposit has been obtained, the article is removed, rinsed in cold and hot water successively, and then air dried. The deposits thus obtained are tough and of pleasing appearance and are 10 more resistant to corrosion and abrasion than any hitherto obtained in the art, and are found to contain a small percentage of mercury.

From tests made by us with and without 15 mercury in the bath (either from the anode or  $\frac{1}{10}$  oz. of mercuric oxide added to the above bath) the effect of the mercury is to cause the voltage drop to increase, resulting in faster and greater deposition of metal coating 20 and less decomposition of electrolyte and loss of hydrogen at the cathode. The effect is also not that of a cathode depolarizer, but is to actually raise the cathode potential up to such value that zinc is deposited rather 25 than hydrogen released. In other words, there is an increased over voltage effect set up by the mercury at the cathode, which reduces hydrogen deposition and increases the zinc and mercury deposition by the equivalent 30 electrochemical amount.

We do not limit ourselves to the particular proportions and percentages herein specified, but the effect of too much mercury is to produce a brittle coating.

35 We do not claim broadly herein the addition of mercury to an alkaline zinc plating bath containing cyanide, as same is claimed broadly in a prior application filed by us December 3, 1921, Serial Number 40 519,765, but we do intend to claim broadly the incorporation of mercury into the anode for the purposes of the process herein described.

We are aware that it has heretofore been 45 proposed to amalgamate zinc anodes for acid zinc plating baths with mercury as well as zinc electrodes for primary batteries, but are not aware that mercury has been before known or used in a zinc anode to increase 50 the over voltage of the cathode in an alkaline zinc plating bath containing cyanide, and therefore do not restrict ourselves except as required by the scope of the appended claims.

55 The replenishment of mercury automatically by solution from the anode as required, while maintaining a substantially constant amount of mercury in solution, is especially

advantageous in practice because it obviates the necessity of making chemical tests of the bath from time to time, as the operator simply has to carry on the process in the ordinary way and gives no attention to the mercury. The bath can be run for a number of weeks without attention and with uniformity of result. Cast iron articles are plated as well as steel and wrought iron articles, even in depressions and irregularities, whereas satisfactory results with cast iron in baths of this character have heretofore only been obtained with difficulty if at all.

What we claim is:

1. The method of zinc electroplating in a bath containing cyanide which consists in making the article to be plated the cathode, 75 and providing an anode containing a substance which enters into the bath and increases the over voltage of the cathode.

2. The method of zinc electroplating in a bath containing cyanide which consists in 80 making the article to be plated the cathode, and providing an anode containing such percentage of a substance which enters into the bath and increases the over voltage of the cathode while remaining in substantially 85 constant percentage in the bath.

3. The method of zinc electroplating in a bath containing cyanide which consists in making the article to be plated the cathode, and providing an anode containing a substance which enters into the bath and increases the over voltage of the cathode while 90 remaining in substantially constant percentage in the bath.

4. The method of zinc electroplating in a 95 bath containing cyanide which consists in making the article to be plated the cathode, and providing an anode containing mercury.

5. The method of zinc electroplating in a 100 bath containing cyanide which consists in making the article to be plated the cathode, and providing an anode containing approximately 1% of mercury.

6. An anode for a cyanide zinc plating 105 bath composed of zinc and a small percentage of mercury.

7. An anode for a cyanide zinc plating bath composed of zinc and approximately 1% of mercury.

Signed at Perth Amboy, in the county of Middlesex and State of New Jersey, this 22d day of December A. D. 1921.

CHARLES H. PROCTOR.  
CHRISTIAN JOHN WERNLUND.